

## UNITED STATES PATENT OFFICE

2,542,161

MINERAL OIL LUBRICANT CONTAINING  
PHOSPHORIZING AND SULFURIZED  
GLYCERYL TRIOLEATEJoseph B. Stucker, Oak Park, Ill., assignor to The  
Pure Oil Company, Chicago, Ill., a corporation  
of OhioNo Drawing. Application March 9, 1946,  
Serial No. 653,438

8 Claims. (Cl. 252—46.6)

1

This invention relates to lubricants and lubricant additives, and more particularly to additives which have the ability to carry high loads and which when blended with mineral lubricating oils give blends having low pour characteristics.

In Patent No. 2,211,306 there is disclosed and claimed a process for making an extreme pressure lubricant additive by sulfurizing a fatty body or fatty oil, and then phosphorizing the sulfurized product. Extreme pressure additives made in accordance with the aforesaid patent have been in successful use for many years and have proved to be highly satisfactory. Such additives when made from ordinary fatty oil, such as lard oil, have one drawback, namely, that the lubricant which results from blending the additive with the mineral oil does not have a sufficiently low pour point.

I have discovered that sulfurized and phosphorized extreme pressure additives having high load carrying characteristics and low pour point characteristics can be prepared in accordance with the method disclosed and claimed in Patent No. 2,211,306 if the fatty body is an ester of a polyhydroxy alcohol and a mono-ethenoid acid of the general formula  $C_nH_{2n-2}O_2$  containing from 10 to 24 carbon atoms in the molecule. As examples of esters which are suitable in preparing additives in accordance with my invention may be mentioned polyhydric alcohol esters of decanoic, myristoleic, palmitoleic, oleic, erucic, and tetracosenoic acids combined with any one of the polyhydroxy alcohols, glycol, glyceryl and sorbitol. Although I prefer those esters which are completely esterified, esters in which only partial esterification has taken place are also suitable. For example, the mono-, di- and tri-esters of glycerol, or mixtures of the three may be used.

Instead of using pure esters of polyhydroxy alcohols and mono-ethenoid acids, compositions may be used which are substantially free of or contain very small amounts of polyethenoid acids or esters thereof and a small amount of ethenoid radicals. For example, partially hydrogenated sunflower, corn and rape seed oil in which the hydrogenation is carried to a point only where the acid radicals having more unsaturation than

2

a single double bond are hydrogenated to a single double bond radical may be used. Olive oil is fairly satisfactory as a starting material. In general, the fatty acid content of compositions useful as starting materials in accordance with my invention should not be less than 80% of mono-ethenoid acids and not more than 10% of acids of greater unsaturation.

In order to demonstrate the invention a composition was prepared by mixing 5 parts by weight of Gulf Coast mineral oil (having a Saybolt viscosity at 100° F. of 200 to 210 seconds, and at 210° F. of 43 to 45 seconds) and 87.6 parts by weight of glyceryl oleates composed of approximately 70% by weight of glyceryl trioleate, 20% by weight of glyceryl dioleate and 10% by weight of glyceryl mono-oleate. The mixture was slowly heated to a temperature of approximately 270° F., whereupon 7.4 parts by weight of finely ground flowers of sulfur were added over a period of about 10 minutes. After the addition of the sulfur was completed the mixture was raised to a temperature of approximately 330° to 340° F. and held at this temperature with constant agitation until a copper strip immersed therein for a period of 2 minutes showed no black coating. This required approximately 7 hours. The mixture was then cooled rapidly to approximately 150° F. and then allowed to cool slowly to room temperature. To 99.6 parts of the sulfurized base thus prepared was added 0.4 part by weight of finely divided phosphorus sesquisulfide and the mixture heated with constant agitation to a temperature of approximately 220° to 230° F. The heating was continued for a period of approximately 5 hours and then allowed to cool. The resulting product was non-corrosive to the copper strip test and did not fume when heated to 300° to 350° F. The resulting product was blended in the amount of 18% by weight with mineral oil in order to obtain a blend corresponding to an 80 S. A. E. gravity oil, and another corresponding to a 90 S. A. E. gravity oil. These blends were tested for viscosity, viscosity index, pour point, and Timken test and compared with similar blends of phosphorized-sulfurized lard oil made in accordance with the specific example set forth in the manner just described in which

glyceryl oleates were used. The results of these tests are set forth in the following table:

Table

| Composition by Wt.                         | Saybolt Vis. at 100° F. | Saybolt Vis. at 210° F. | V. I. | Pour | Timken Test              |
|--------------------------------------------|-------------------------|-------------------------|-------|------|--------------------------|
| 18% S-P Lard Oil                           |                         |                         |       |      |                          |
| 41% 100 Gulf Coast Pale Oil                | 353                     | 59.8                    | 116   | +10  | 71 lbs., 39,500 p. s. i. |
| 41% 200 Gulf Coast Pale Oil                |                         |                         |       |      |                          |
| 18% S-P glyceryl oleate                    | 308                     | 56.8                    | 123   | -30  | 77 lbs., 39,500 p. s. i. |
| 82% 100 Gulf Coast Pale Oil                |                         |                         |       |      |                          |
| 18% S-P Lard Oil                           |                         |                         |       |      |                          |
| 41% 200 Gulf Coast Pale Oil                | 1,248                   | 91.1                    | 79    | +5   | 68 lbs., 35,000 p. s. i. |
| 41% 160 vis. @ 210 Gulf Coast bright stock |                         |                         |       |      |                          |
| 18% S-P glyceryl oleate                    |                         |                         |       |      |                          |
| 63% 200 Gulf Coast Pale Oil                | 924                     | 86.1                    | 98    | -20  | 86 lbs., 38,000 p. s. i. |
| 19% 160 vis. @ 210 Gulf Coast bright stock |                         |                         |       |      |                          |

From an inspection of the table it is apparent that the blends made by sulfurizing and phosphorizing the glyceryl oleate had higher viscosity indexes than the sulfurized-phosphorized lard oil blends, and that the pour points of the sulfurized-phosphorized glyceryl oleate blends were considerably lower. Note for example that the 90 S. A. E. grade (the last sample in the table) had a pour point 30° lower than the 80 S. A. E. grade made from the lard oil (the first sample in the table). Note also that the Timken tests for the sulfurized-phosphorized glyceryl oleate compositions were at least as good as the sulfurized-phosphorized lard oil compositions, and in general, were superior from a load carrying standpoint.

BLENDS prepared in accordance with the second and fourth samples in the table were subjected to actual service tests in the transmission and differential of a number of different automobiles. After 4,000 to 5,000 miles running the gears showed no evidence of wear, and the lubricant exhibited high stability. Low temperature characteristics of the lubricant were excellent as evidenced by the fact that after the automobile had been allowed to stand outdoors at temperatures approaching -10° F. the gears could be shifted with ease.

In preparing the additive in accordance with my invention sulfurization may be effected by means of elemental sulfur in an amount of from 1 to 10% by weight, and preferably 5 to 8.5% by weight of sulfur based on the sulfurized product, or by means of sulfur chloride in accordance with the method disclosed in Patent No. 2,352,818 in the amount of approximately 5 to 15% by weight of the sulfur chloride based on the ester. The phosphorization step is preferably effected by means of phosphorus sesquisulfide at temperatures of about 220° to 230° F., but other phosphorus compounds, including halides such as phosphorus trichloride, oxyhalides such as phosphorus oxychloride, sulfides, such as phosphorus pentasulfide, oxides such as phosphorus pentoxide, as well as elemental phosphorus compounds such as tin phosphide, may be used. The amount of phosphorus in the base should not exceed 2%, and preferably should be only a fraction of 1%, preferably 0.2 to 0.6% based on the weight of the sulfurized base.

It will be seen, therefore, that by sulfurizing and phosphorizing a fatty body composed chiefly of esters of polyhydroxy alcohols and mono-ethenoid acids a lubricant additive having high load characteristics and unexpected low temperature characteristics can be obtained. Additives made in accordance with my invention may be used in lubricating oils in amounts ranging from

approximately 0.5 to 20% or more by weight of the finished lubricant. The amount will depend

upon the service for which the lubricant is intended. Although additives prepared in accordance with my invention may be blended with all types of mineral lubricating oil, I prefer to keep the amount of Pennsylvania bright stock present in the blend to a minimum since these stocks tend to cause separation of the additive from the oil.

It is claimed:

1. A lubricant additive substantially consisting of the reaction product of phosphorus sesquisulfide and sulfurized glyceryl oleates, at least 70% of said glyceryl oleates being glyceryl trioleate, the sulfur content of said additive being about 1 to 10 per cent, and the phosphorus content thereof being about 0.2 to 0.6 per cent by weight.

2. A lubricant additive in accordance with claim 1 in which the sulfur content is 5 to 8.5 per cent by weight.

3. A lubricant additive in accordance with claim 1 in which the glyceryl oleates are composed of mono-, di- and tri-glyceryl oleates.

4. A lubricant additive substantially consisting of the product resulting from the reaction of sulfur and glyceryl oleates containing at least 70% of glyceryl trioleate, followed by reaction with phosphorus sesquisulfide, said product containing about 5 to 8.5 per cent by weight of sulfur and about 0.2 to 0.6 per cent by weight of phosphorus.

5. A lubricant additive substantially consisting of the product resulting from the reaction of about 5 parts by weight of mineral lubricating oil, 87.5 parts by weight of glyceryl oleates containing at least 70% of glyceryl trioleate, and 7.4 parts by weight of sulfur, followed by reaction with about 0.4 part by weight of phosphorus sesquisulfide.

6. A mineral lubricating oil containing as the principal extreme pressure additive from 0.5 to 20 per cent by weight of the additive defined by claim 1, said oil having the ability to flow at temperatures approaching -10° F.

7. A lubricating oil of S. A. E. 80 grade composed of Gulf Coast lubricating oil to which has been added as the principal extreme pressure additive from 0.5 to 20 per cent of the additive defined by claim 1, said oil having a pour point of about -30° F.

8. A lubricating oil of S. A. E. 90 grade composed of Gulf Coast lubricating oil containing as the principal extreme pressure additive from 0.5 to 20 per cent by weight of the additive defined by claim 1, said oil having a pour point of about -20° F.

JOSEPH B. STUCKER.

**5****REFERENCES CITED**

The following references are of record in the  
file of this patent:

**UNITED STATES PATENTS**

| Number    | Name            | Date          |
|-----------|-----------------|---------------|
| 2,211,306 | Whittier et al. | Aug. 13, 1940 |
| 2,237,096 | Dearborn        | Apr. 1, 1941  |

**6**

| Number    | Name           | Date          |
|-----------|----------------|---------------|
| 2,262,813 | Morway et al.  | Nov. 18, 1941 |
| 2,308,427 | Roehner et al. | Jan. 12, 1943 |
| 2,355,106 | Prutton        | Aug. 8, 1944  |
| 2,441,587 | Musselman      | May 18, 1948  |
| 2,480,873 | Musselman      | Sept. 6, 1949 |
| 2,483,571 | Brennan        | Oct. 4, 1949  |